# EUROPEAN PATENT SPECIFICATION

(11) **EP 3 431 305 B1**
(45) Date of publication and mention of the grant of the patent: **26.08.2020**
(21) Application number: 18184788.0
(22) Date of filing: 20.07.2018
(51) Int. Cl.: B42D 25/41, B42D 25/378

(54) **A DOCUMENT SECURITY ELEMENT, A VALUE DOCUMENT WITH A SECURITY ELEMENT AND A METHOD OF MANUFACTURING OF A VALUE DOCUMENT**
DOKUMENTSICHERHEITSELEMENT, EIN WERTDOKUMENT MIT EINEM SICHERHEITSELEMENT UND EIN VERFAHREN ZUR HERSTELLUNG EINES WERTDOKUMENTS
ÉLÉMENT DE SÉCURITÉ DE DOCUMENT, DOCUMENT DE VALEUR AVEC UN ÉLÉMENT DE SÉCURITÉ ET PROCÉDÉ DE FABRICATION D'UN DOCUMENT DE VALEUR

(30) Priority: 21.07.2017 PL 42230017
(43) Date of publication of application: 23.01.2019
(73) Proprietor: Polska Wytwornia Papierow Wartosciowych S.A., 00-222 Warszawa (PL)
(72) Inventor: Wójcik, Pawel, 03-185 Warszawa (PL); Gurtowska, Joanna, 03-043 Warszawa (PL); Wojciechowska, Agata, 02-791 Warszawa (PL); Biernacki, Ariel, 03-193 Warszawa (PL); Leszczynska-Ambroziewicz, Ewa, 05-200 Wolomin (PL)
(74) Representative: Górska, Anna

(56) References cited:
- WO-A1-03/056507
- WO-A2-98/22291
- US-A1- 2015 306 887

## Description

### Field of the invention

The object of the invention is an element securing a document with an image invisible in visible light, and visible in the infrared, and a value document, such as a banknote, certificate, visa, passport, identity card or other, comprising a security element. Furthermore, the object of the invention is also a method of manufacturing of such a value document.

### Background of the invention

Value documents may comprise various security features, such as watermark, microprint, convex print, etc. However, new types of security features are still being introduced which allow them to be better protected against forgery.

For example, US Patent Application No. US2008088859A describes an invention relating to a value document, particularly a banknote, which has an individualising mark - in particular, constituting a number - created on the document in a contactless manner by means of a laser. The identification mark can be created on both sides of the value document by means of properly directed laser beams placed on one side of the document.

Canadian Patent Application No. CA2645578A presents a method for producing a data carrier in the form of e.g. a banknote that comprises an identifier in the form of patterns, letters, digits or an image. The identifier - in the solution being the object of the invention - is recognised visually or by means of appropriate devices designed for detecting security features. To apply the identifier onto the document, short laser pulses are used which modify the substance sensitive to the laser beam at a specific wavelength. Document WO 98/22291 discloses a document security element according to the preamble of claim 1.

The aim of the invention was to develop methods for securing documents, alternative to those present in the prior art, which would ensure a higher level of document security, making forgery more difficult. The invention will allow for application of images invisible to the naked eye, as well as repeated personalised data, numbering or time stamps.

### Essence of the invention

The essence of the invention is a document security element comprising an image invisible in visible light, and visible in the infrared in the 700-1000 nm range, characterised in that it includes a layer of paper susceptible to laser engraving, covered with a layer of paint transparent in infrared radiation, wherein the layer of paper comprises an engraving made using a laser beam pulse, performed after covering the layer of paper with the layer of paint.

The invention also includes a value document comprising a security element, in particular a document constituting a banknote, certificate, visa, passport or an identity card, characterised in that it comprises a document security element, described above in the essence of the invention, comprising an image invisible in visible light and visible in the infrared.

In addition, the solution according to the invention also relates to a method of manufacturing of a value document comprising an image invisible in visible light and visible in the infrared, characterised in that the layer of paper susceptible to laser engraving is covered with a layer of paint, wherein the paint is transparent in the infrared, and then the layer of paper susceptible to engraving is subjected to a laser beam pulse at a wavelength of 1064 nm at the place of paint application in such a manner that the layer of paint remains intact.

Preferably, the layer of paper susceptible to laser engraving is covered with the layer of paint in a printing process.

Also preferably, the colour and/or thickness of the paint by means of which the paper susceptible to engraving is covered provides adequate coverage of marked elements, i.e. such that the engraved element is not visible in daylight.

Preferably, the paint by means of which the paper susceptible to engraving is covered is a paint chosen from the following: intaglio, offset, screenprint or flexographic paints, and particularly preferably the thickness of the layer for the intaglio paint is between 40 µm and 60 µm, and for the screenprint paint it is between 15 µm and 20 µm, while for flexographic paint it is between 5 µm and 30 µm, and for the offset paint at least two of the partial optical densities measured for cyan, magenta, yellow colours are at least 0.8, or the partial optical density measured for black colour is at least 0.7.

Preferably, in the method according to the invention, the source of the laser beam is a Nd:YAG neodymium laser.

Also preferably, the power of the laser beam pulse ranges from 1.1 ^{∗} 10¹⁴ to 1.8^{∗} 10¹⁴ W/m², the beam speed ranges from 30 to 1000 mm/s, and the pulse frequency ranges from 700 to 15,000 Hz.

The object of the invention is presented in examples which do not limit its scope and in the drawing, in which:
Fig. 1 illustrates a cross-section of a document which is the object of the invention,
Fig. 2 illustrates an image visible in visible light,
Fig. 3 a-c illustrate images visible in the infrared at a wavelength greater than 700 nm on various types of value documents.

### Embodiments

In an embodiment, value document 10, the cross-section of which is illustrated in Fig. 1, comprises a base layer of paper 11 made of cotton, cellulose and semi-cellulose. This layer is susceptible to engraving by means of a Nd:YAG laser beam with a wavelength of 1064 nm.

The paper susceptible to engraving of the embodiment comprises a paper substrate layer which is covered with a coating layer. The paper substrate layer comprises a laser pigment of tin dioxide doped with antimony oxide, and titanium white. In turn, the coating layer comprises a laser pigment of tin dioxide doped with antimony oxide. Both, paper in which the paper substrate layer was covered with the coating layer on one side only, and paper in which the paper substrate layer was covered with the coating layer on both sides were used. In the paper used, the laser pigment of tin dioxide doped with antimony oxide comprised from 95% to 99% by weight of tin dioxide (SnO₂) and from 1% to 5% by weight of antimony oxide (Sb₂O₃). This pigment allows for obtaining particularly legible and clear laser-engraved markings. The titanium white used was a rutile form of titanium dioxide (TiO₂). In turn, the paper substrate layer comprised conventional fibres and additives.

The paper substrate layer comprises 2.5-10%, preferably 5% by weight of laser pigment of tin dioxide doped with antimony oxide and from 2.5% to 10%, preferably 3.5% by weight of titanium white. The coating layer comprises 0.5-3%, preferably 2% by weight, of laser pigment of tin dioxide doped with antimony oxide.

A graphic layout is applied onto the base layer of paper 11 by means of typical printing techniques, such as, among others, offset, screenprint, intaglio or flexographic techniques. In the embodiment, an additional layer of paint 12 was applied onto a selected portion of the base layer 11 of the value document 10, which constitutes a pattern made with infrared-transparent paint, wherein various paints used in the above-mentioned printing techniques can be used. Various paint thicknesses were tested depending on the above-mentioned techniques, and the results are presented in Table 1.

**Table 1**

| **Type of paint** | **Min. thickness of the paint layer [µm]** | **Max. thickness of the paint layer [µm]** | **Optimal thickness of the paint layer [µm]** |
|---|---|---|---|
| Intaglio paint | 10 | 60 | 40-60 |
| Screenprint paint | 10 | 40 | 15-20 |
| Flexographic paint | 5 | 30 | 5-30 |
| Offset paint | at least two of the partial optical densities measured for cyan, magenta, yellow colours are at least 0.8, or the partial optical density measured for black colour is at least 0.7. | | |

After printing the additional layer 12 on the base layer of paper 11, the value document 10 was subjected to the process of laser engraving by means of a Nd:YAG neodymium laser with a wavelength of 1064 nm, which creates an image 13 in sepia or in shades of grey. Engraving by means of a laser beam was done in such a manner that the engraved image 13 was created under the additional layer 12 of infrared-transparent paint. The additional layer 12 of paint was not affected by the laser beam. The image 13 obtained in this manner was visible in the infrared at a wavelength above 700 nm, while the image was invisible in visible light.

In the embodiment, in order to apply the additional layer 12, intaglio, offset, screenprint or flexographic infrared-transparent paints were used with their colouring and/or thickness ensuring adequate coverage of the elements marked with the laser beam. Thanks to the use of covering colours and/or appropriate thickness of paint 12, the engraved image 13 is invisible in visible light (Fig. 2).

In visible light, on the value document 10 obtained by the method according to the invention, an image is visible which constitutes the additional layer 12 printed with paint, while the engraved image 13 remains hidden. When the value document 10 is placed in the infrared at a wavelength above 700 nm, then only the engraved image 13 which absorbs the infrared is visible.

It is possible to use the method that is the object of the invention to apply hidden images onto various types of value documents. Hidden images can be, e.g., alphanumeric data or time stamps, bitmap pixel graphics and vector graphics.

An exemplary use of the method according to the invention is shown in Fig. 3a, where the value document 10 is a banknote and the hidden image 13 - visible in the infrared, made with the laser engraving technique - comprises the banknote's number. This number may constitute a repetition of traditional numbering of banknote made e.g. with a typographic technique. In turn, Fig. 3b shows a value document constituting a personalised secured document (e.g. ID card, visa or certificate), where the hidden image 13, visible in the infrared, comprises a photograph. By applying a repeated photograph of the document's holder with a technique other than in case of the main photograph visible in daylight, the level of personalisation security increases. In turn, Fig. 3c shows, for example, the value document 10 in the form of a passport, where a special code (e.g. time stamp) was applied with the laser engraving technique.

## Claims

1. A document security element comprising an image invisible in visible light, and visible in the infrared in the 700-1000 nm range, **characterised in that** it includes a layer of paper (11) susceptible to laser engraving, covered with a layer of paint (12) transparent in infrared radiation, wherein the layer of paper (11) comprises an engraving made by means of a laser beam pulse, performed after covering the layer of paper (11) with the layer of paint (12).

2. A value document comprising a security element, especially a document constituting a banknote, certificate, visa, passport or an identity card, **characterised in that** it comprises the element securing the document comprising an image invisible in visible light and visible in the infrared, defined in claim 1.

3. A method of manufacturing of the value document defined in claim 2, **characterised in that** the layer of paper (11) susceptible to laser engraving is covered with the layer of paint (12), wherein this paint is transparent in the infrared, and then the layer of paper (11) susceptible to engraving is subjected to a laser beam pulse at a wavelength of 1064 nm at the place of paint application in such a manner that the layer of paint (12) remains intact.

4. The method according to claim 3, **characterised in that** the layer of paper (11) susceptible to laser engraving is covered with the layer of paint (12) in the printing process.

5. The method according to claims from 3 to 4, **characterised in that** the colouring and/or thickness of the paint by means of which the paper (11) susceptible to engraving is covered provides adequate coverage of marked elements.

6. The method according to claims from 3 to 5, **characterised in that** the paint by means of which the paper (11) susceptible to engraving is covered is a paint chosen from the following: intaglio, offset, screenprint or flexographic paints.

7. The method according to claim 6, **characterised in that** the thickness of the layer (12) for intaglio paint is between 40 µm and 60 µm.

8. The method according to claim 6, **characterised in that** the thickness of the layer (12) for screenprint paint is between 15 µm and 20 µm.

9. The method according to claim 6, **characterised in that** the thickness of the layer (12) for flexographic paint is between 5 µm and 30 µm.

10. The method according to claim 6, **characterised in that** in case of the applied layer (12) of offset paint, at least two of the partial optical densities measured for cyan, magenta, yellow colours are at least 0.8, or the partial optical density measured for black colour is at least 0.7.

11. The method according to claim 3, **characterised in that** the source of the laser beam is a Nd:YAG neodymium laser.

12. The method according to claim 3, **characterised in that** power of the laser beam pulse ranges from 1.1 ^{∗} 10¹⁴ to 1.8^{∗} 10¹⁴ W/m², the beam speed ranges from 30 to 1000 mm/s, and the pulse frequency ranges from 700 to 15,000 Hz.

## Patentansprüche

1. Ein Dokumenten-Sicherheitselement, umfassend ein Bild, das im sichtbaren Licht unsichtbar und im Infrarot im Bereich von 700-1000 nm sichtbar ist, **dadurch gekennzeichnet, dass** es eine Papierschicht (11) beinhaltet, die für eine Lasergravur anfällig ist, die mit einer in Infrarotstrahlung transparenten Farbschicht (12) bedeckt ist, wobei die Papierschicht (11) eine Gravur umfasst, die mittels eines Laserstrahlpulses durchgeführt wird, nachdem die Papierschicht (11) mit der Farbschicht (12) bedeckt worden ist.

2. Ein Wertdokument, umfassend ein Sicherheitselement, insbesondere ein Dokument, das eine Banknote, ein Zertifikat, ein Visum, einen Reisepass oder einen Personalausweis bildet, **dadurch gekennzeichnet, dass** es ein Element umfasst, das das Dokument sichert, umfassend ein Bild, das im sichtbaren Licht unsichtbar und im Infrarot sichtbar ist, definiert in Anspruch 1.

3. Ein Verfahren zur Herstellung des in Anspruch 2 definierten Wertdokuments, **dadurch gekennzeichnet, dass** die für die Lasergravur anfällige Papierschicht (11) mit der Farbschicht (12) bedeckt wird, wobei diese Farbe im Infrarot transparent ist, und dann die gravierbare Papierschicht (11) einem Laserstrahlpuls bei einer Wellenlänge von 1064 nm am Ort der Farbaufbringung derart ausgesetzt wird, dass die Farbschicht (12) intakt bleibt.

4. Ein Verfahren nach Anspruch 3, **dadurch gekennzeichnet, dass** die lasergravierbare Papierschicht (11) im Druckverfahren mit der Farbschicht (12) bedeckt wird.

5. Ein Verfahren nach den Ansprüchen von 3 bis 4, **dadurch gekennzeichnet, dass** die Färbung und/oder Dicke der Farbe, mit der das gravierbare Papier (11) bedeckt ist, eine ausreichende Abdeckung der markierten Elemente gewährleistet.

6. Ein Verfahren nach den Ansprüchen von 3 bis 5, **dadurch gekennzeichnet, dass** die Farbe, mit der das gravierbare Papier (11) bedeckt ist, eine der folgenden Farben ist: Intaglio-, Offset-, Siebdruck- oder Flexofarbe.

7. Ein Verfahren nach Anspruch 6, **dadurch gekennzeichnet, dass** die Dicke der Schicht (12) für Intagliofarbe zwischen 40 µm und 60 µm liegt.

8. Verfahren nach Anspruch 6, **dadurch gekennzeichnet, dass** die Dicke der Schicht (12) für Siebdruckfarbe zwischen 15 µm und 20 µm liegt.

9. Ein Verfahren nach Anspruch 6, **dadurch gekennzeichnet, dass** die Dicke der Schicht (12) für Flexodruckfarbe zwischen 5 µm und 30 µm liegt.

10. Ein Verfahren nach Anspruch 6, **dadurch gekennzeichnet, dass** bei der aufgebrachten Schicht (12) aus Offsetfarbe mindestens zwei der für Cyan, Magenta, Gelb gemessenen partiellen optischen Dichten mindestens 0,8 betragen oder die für Schwarz gemessene partielle optische Dichte mindestens 0,7 beträgt.

11. Ein Verfahren nach Anspruch 3, **dadurch gekennzeichnet, dass** die Quelle des Laserstrahls ein Nd:YAG-Neodym-Laser ist.

12. Ein Verfahren nach Anspruch 3, **dadurch gekennzeichnet, dass** die Leistung des Laserstrahlpulses von 1,1 ^{∗} 10¹⁴ bis 1,8^{∗}10¹⁴ W/m², die Strahlgeschwindigkeit von 30 bis 1000 mm/s und die Pulsfrequenz von 700 bis 15.000 Hz beträgt.

## Revendications

1. Un élément de sécurité de document comprenant une image invisible à la lumière visible et visible à l'infrarouge dans la plage de 700 à 1000 nm, **caractérisé en ce qu'**il comprend une couche de papier (11) susceptible d'être gravée au laser, recouverte d'une couche de peinture (12) transparente dans le rayonnement infrarouge, dans lequel la couche de papier (11) comprend une gravure réalisée au moyen d'une impulsion de faisceau laser, effectuée après avoir recouvert la couche de papier (11) avec la couche de peinture (12).

2. Un document de valeur comprenant un élément de sécurité, notamment un document constituant un billet de banque, un certificat, un visa, un passeport ou une carte d'identité, **caractérisé en ce qu'**il comprend l'élément assurant la sécurité du document comprenant une image invisible à la lumière visible et visible à l'infrarouge, défini dans la revendication 1.

3. Une méthode de fabrication du document de valeur défini dans la revendication 2, **caractérisée en ce que** la couche de papier (11) susceptible d'être gravée au laser est recouverte avec la couche de peinture (12), cette peinture étant transparente à l'infrarouge, et puis la couche de papier (11) susceptible d'être gravée est soumise à une impulsion de faisceau laser à une longueur d'onde de 1064 nm sur le lieu d'application de la peinture de manière à ce que la couche de peinture (12) reste intacte.

4. La méthode selon la revendication 3, **caractérisée en ce que** la couche de papier (11) susceptible d'être gravée au laser est recouverte avec la couche de peinture (12) dans le processus d'impression.

5. La méthode selon les revendications de 3 à 4, **caractérisée en ce que** la coloration et/ou l'épaisseur de la peinture au moyen de laquelle le papier (11) susceptible d'être gravé est recouvert assure une couverture adéquate des éléments marqués.

6. La méthode selon les revendications de 3 à 5, **caractérisée en ce que** la peinture au moyen de laquelle le papier (11) susceptible d'être gravé est recouvert est une peinture choisie parmi les suivantes: peintures pour intaglio, offset, sérigraphie ou flexographie.

7. La méthode selon la revendication 6, **caractérisée en ce que** l'épaisseur de la couche (12) pour peinture pour intaglio sur acier est comprise entre 40 µm et 60 µm.

8. La méthode selon la revendication 6, **caractérisée en ce que** l'épaisseur de la couche (12) pour peinture sérigraphique est comprise entre 15 µm et 20 µm.

9. La méthode selon la revendication 6, **caractérisée en ce que** l'épaisseur de la couche (12) pour peinture flexographique est comprise entre 5 µm et 30 µm.

10. La méthode selon la revendication 6, **caractérisée en ce que** dans le cas de la couche appliquée (12) de peinture offset, au moins deux des densités optiques partielles mesurées pour les couleurs cyan, magenta, jaune sont d'au moins 0,8 ou la densité optique partielle mesurée pour la couleur noire est d'au moins 0,7.

11. La méthode selon la revendication 3, **caractérisée en ce que** la source du faisceau laser est un laser au néodyme Nd:YAG.

12. La méthode selon la revendication 3, **caractérisée en ce que** la puissance de l'impulsion du faisceau laser est comprise entre 1,1 ^{∗} 10¹⁴ et 1,8^{∗}10¹⁴ W/m², la vitesse du faisceau entre 30 et 1000 mm/s et la fréquence des impulsions entre 700 et 15 000 Hz.
